

Nov. 20, 1923.

1,474,888

F. BRINER

## METHOD OF CASTING STEEL FRAMES

Filed Oct. 29, 1920



Patented Nov. 20, 1923.

1,474,888

# UNITED STATES PATENT OFFICE.

FRANK BRINER, OF CHESTER, PENNSYLVANIA, ASSIGNOR TO PENN SEABOARD STEEL CORPORATION, OF NEW YORK, N. Y., A CORPORATION OF NEW YORK.

## METHOD OF CASTING STEEL FRAMES.

Application filed October 29, 1920. Serial No. 420,436.

To all whom it may concern:

Be it known that I, FRANK BRINER, a citizen of the United States, residing in Chester, Pennsylvania, have invented 5 Methods of Casting Steel Frames, of which the following is a specification.

One object of this invention is to provide a novel and commercially practical method of forming the elongated steel side frames 10 of steam and electric locomotives and the invention especially contemplates a method of procedure whereby it is possible to obtain sound, dense castings, free from checks 15 and cracks, as well as from internal stresses set up in cooling and which shall be of such a constitution as to render failure unlikely under conditions of use.

These objects and other advantageous ends I attain as hereinafter set forth, reference 20 being had to the accompanying drawings, in which,

Fig. 1 is a vertical section on the line 1—1, Fig. 2, showing a mold with the casting 25 therein made in accordance with my invention; Fig. 2 is a plan of the mold shown in Fig. 1; and

Figs. 3 and 4 are respectively an end elevation and a transverse vertical section on the line 4—4, Fig. 2.

In casting the elongated trussed structures commonly known as side frames in locomotive structures, I have discovered that the best results can be obtained if the mold be 35 so constructed and positioned that said frames are cast in a vertical, rather than a horizontal plane, and the best product is obtained if each frame be cast with the top frame member occupying the highest position in the mold.

In carrying out my invention therefore, I provide a narrow, elongated mold box having two outside sections 1 and 2 and an intermediate section 3, all relatively thin and mounted in engagement with each other in parallel vertical planes. The frame pattern is placed in the intermediate section 3 and after the sand or equivalent molding material has been properly packed around it, is drawn therefrom, sand being also packed in the two outside sections 1 and 2, and the whole assembled so that when ready for the molten metal to be poured into the same, the plane of the metal-receiving cavities or the plane of the frame itself is vertical.

In a typical case the frame would consist of a relatively straight top member 4, a bottom member 5 substantially parallel therewith, an inclined end member 6 connecting one end of the bottom member 5 with the extended adjacent end of the top member 4, an end member 7, inclined members 8 and 9 connecting the end member with the top and bottom members 4 and 5 respectively, and three pairs of pedestal legs 10—10, 10<sup>a</sup>—10<sup>a</sup>, 65 and 10<sup>b</sup>—10<sup>b</sup>, extending from the top to the bottom member in substantially parallel relation. A bracing member 20 also connects the members 4 and 5 between the adjacent pedestal members 10 and 10<sup>a</sup>.

In accordance with my invention a riser or feeder-head 21 is provided for the full length of the top rail or frame member 4 and a gate 11 is provided whereby the molten steel is delivered to the mold at one end of the end member 7, there being also a riser 12 from the middle of said end member.

It is particularly to be noted that in accordance with my invention, the sand cores 14—19, 22 and 23 between the frame members 5 and 4, as well as the cores 24 and 25 between the pedestal legs 10, are made hollow, and preferably have their cavities filled with elastic or yieldable material such as hay, or the like which will not interfere with the contraction of the adjacent bodies of metal as would be the case if unyielding solid cores were employed.

When the molten steel is supplied to the gate 11, it first fills the space defining the bottom member 5 and thereafter rises through the pedestal legs and inclined members 6 and 8, ultimately filling the space for the top member 4, and the riser cavities 12 and 21. There is thus provided in said risers a mass of molten metal with sufficient heat capacity to insure a full supply of metal to the bottom and substantially vertical frame members during cooling of the casting, the metal in the continuous deep riser 21 preventing the cooling stresses otherwise occurring as said casting solidifies. As a consequence of this method of procedure the lowermost member as well as the top and vertical members of the frame have been found to be invariably sound and dense.

The mass of metal in the riser cavity 21 moreover serves as a reinforcement to the top member 4 in holding the pedestal legs 10, 10<sup>a</sup> and 10<sup>b</sup> together in their proper lo-

cation and avoids the cracking or checking which has hitherto been found to occur at or adjacent to the points where they join the said member 4, preventing also the internal stresses which at these same points have been found to cause failure under conditions attending their use on locomotives. The tendency to crack or check is likewise reduced or prevented by the use of the hollow yielding cores 14-18 which, owing to their inherent elasticity or to the burning out of their combustible contents, permit the contraction of the cooling metal in the various frame members, without setting up injurious internal stresses.

It is further noted that the riser heads 12 and 21 are wholly outside of the pedestal cavities so that the presence of sound metal in the pedestal legs as well as in the inclined and end members is assured owing to the rising of any foreign material through and out of them into the mass within the cavity for the head. Moreover, by casting the frame in a vertical plane, the amount of sand cracked or spalled off of the cores by the action of the heat as the metal flows into the mold, is at a minimum, and in any case what few particles are present, float into the riser cavities 12 and 21, so that the frame members, particularly the member 4 which constitutes the top member of the frame, will be found to be sound and perfect in practically every casting made.

The cores between the risers 21 and 12 and between the latter and the gate 11 are also preferably made hollow and filled with straw or the like so that the finished casting 30 is not only uniformly dense and homogeneous in all its members but is free from all internal stresses—the procedure above defined having been found to permit of the full unrestricted natural shrinkage of the metal during cooling without the production of imperfect castings.

I claim:

1. The method of casting a locomotive side frame which consists in forming a mold of the frame, with a riser cavity co-extensive with one of the longitudinal members thereof; and pouring the casting with the cavities defining the frame in a vertical plane and below the riser cavity.

2. The method of casting a locomotive side frame which consists of forming a mold of

the frame with hollow cores between the cavities for its vertical members; and pouring the casting with the frame defining cavities in a vertical plane.

3. The method of casting the side frame of a locomotive which consists in forming a mold of the frame with a riser cavity co-extensive with and above the top frame member; and pouring the casting with the cavity defining the frame in a vertical plane.

4. The method of casting a locomotive side frame which consists in forming a mold of said frame with yieldable cores between the longitudinally extending frame members and a riser cavity co-extensive with and above the top frame member; and pouring the casting with the mold in position to cause the molten metal to successively fill the cavity defining the bottom member of the frame, the cavities defining the pedestal legs and the riser cavity.

5. The method of casting a locomotive side frame which consists in forming a mold of the frame with a riser cavity coextensive with one of the longitudinal frame members; and pouring the molten metal of the casting into the cavity of one of the end frame members with the mold in position to cause the molten metal to successively fill the cavity for the bottom longitudinal frame member, the cavities for the pedestal legs, the top frame member and the riser cavity above the same.

6. The method of casting a locomotive side frame which consists in forming a mold of the frame with a riser cavity co-extensive with the top frame member, a gate leading into one of the end frame members and a second riser cavity between the gate and said first riser cavity; and pouring the casting with the frame and riser cavities in a vertical plane.

7. The method of casting a locomotive side frame which consists in forming a mold of the frame with a riser cavity co-extensive with the top frame member, a gate leading into one of the end frame members and a second riser cavity between the gate and said first riser cavity; and pouring the casting with the frame and riser cavities in a vertical plane, there being hollow cores between the riser cavities and between the cavities for the vertical frame members.

FRANK BRINER